# EUROPEAN PATENT SPECIFICATION

(11) **EP 2 057 254 B1**
(45) Date of publication and mention of the grant of the patent: **12.01.2011**
(21) Application number: 07789127.3
(22) Date of filing: 06.08.2007
(51) Int. Cl.: C10L 9/10

(54) **COAL WITH IMPROVED COMBUSTION PROPERTIES**
KOHLE MIT VERBESSERTEN VERBRENNUNGSEIGENSCHAFTEN
CHARBON DOTÉ DE PROPRIÉTÉS DE COMBUSTION AMÉLIORÉES

(30) Priority: 12.08.2006 GB 0616094
(43) Date of publication of application: 13.05.2009
(73) Proprietor: Aquafuel Research Limited, Sittingbourne, Kent ME9 8HL (GB)
(72) Inventor: DAY, Paul, Kent ME9 8HL (GB); SIROVSKI, Felix, Kent ME9 8HL (GB); DAUT, Sergej, Kent ME9 8HL (GB)
(74) Representative: Gemmell, Peter Alan
(86) International application number: PCT/GB2007/002991
(87) International publication number: WO 2008/020169

(56) References cited:
- EP-A- 0 252 853
- EP-A- 0 346 100
- GB-A- 518 958
- US-A- 2 460 284
- US-A- 2 460 285

## Description

### BACKGROUND OF THE INVENTION

### 1. Field of the Invention

The present invention relates to a method for improving the combustion properties of a coal, to a coal with improved combustion properties, and to a process for combustion of a coal with reduced emissions.

### 2. Description of the Prior Art

Incomplete combustion in coal fired furnaces results in carbon being retained in ash, and limits the efficiency of coal fired plant. The carbon in ash contributes to the overall ash emission, reduces the efficiency of electrostatic precipitators for ash removal, and makes the ash less easy to dispose of, for example as a component for cement.

Many coal-fired power plants, including Russian and Chinese plants, are using low-grade coals with low reactivity. The main challenges faced when firing these grades of coal are:
- High carbon content in the fly ash: up to 15-20%;
- Significant NOx emission.

The high content of unburned carbon in the fly ash results in the significant heat losses: up to 5% or even higher depending on the coal ash content.

The NOx concentration in effluent gases at air excess (a) of 1.4 is 700-900 mg/m³ (recalculated to NO₂) depending on the boiler power.

EP1498470 lists several methods for reducing carbon in ash from coal burning, including increasing the excess of air introduced with the fuel, or adding metals such as calcium and magnesium. These methods have undesirable effects, with increased air causing higher NOx emissions, and use of metals such as calcium and magnesium requiring large amounts, and causing fouling of the system. EP1498470 proposes the addition of 2-500 ppm of a manganese compound, preferably a manganese tricarbonyl compound.

EP-A-0 252 853 discloses a composite catalyst comprising, on a pyrolysed carbon support, a metal chelate such as iron phthalocyanine. The origin of the pyrolysed carbon support may be fossil but also vegetable. The material comprises 2-25 wt% of the carbon material and 60-90 wt% of a mineral matrix.

US-A-2 460 284 and US-A-2 460 285 are concerned with methods of improving the combustion of tobacco and cigarette paper, respectively, by treating the tobacco or cigarette paper with a porphyrin, preferredly chlorophyll.

### SUMMARY OF THE INVENTION

Aspects of the invention are specified in the independent claims. Preferred features are specified in the dependent claims.

We have found that the invention can provide improved carbon burnout, resulting in reduced carbon content in the ash. The activation energy for oxidation may also be reduced. NOₓ formation in combustion is related to the excess of air over the stoichiometric requirement: more excess means higher NOₓ and lower thermal efficiency. Improved rates of combustion/lower activation energy tends to reduce excess air requirement and lower NOₓ production. The combustion chamber airflow is typically actively managed and can be altered to optimise combustion conditions to minimise carbon content in ash and minimise NOₓ.

The invention is of particular applicability to low-grade coals such as brown coal or bituminous coal.

The metal phthalocyanine of the present invention preferably contains a metal with two or more possible oxidation states. Examples include transition metals such as iron, cobalt or manganese.

The metal phthalocyanine additive may be put up in an aqueous solution and applied to the solid fuel by methods commonly known in the art, for example by spraying onto the solid fuel. Alternately the metal phthalocyanine is applied by sublimation and vapour deposition.

Synthetic phthalocyanines have industrial uses, for example copper phthalocyanlne is widely used as a cyan pigment.

### BRIEF DESCRIPTION OF THE DRAWINGS

The invention will now be further described, by way of example only, with reference to the following drawings, in which:
Figures 1-3 are graphs of, respectively, TG, DTG and DTA results for a coal in accordance with an aspect of the invention and comparative samples;
Figures 4-6 are graphs showing linearised DTG data for, respectively, untreated brown coal, H₂SO₄-treated brown coal and Fe additive treated brown coal;
Figures 7 and 8 are graphs of DTA results for untreated brown coal and for brow coal treated, respectively with an iron-based additive in accordance with the invention and a cobalt-based additive in accordance with the invention;
Figures 9-11 are graphs showing, respectively, TG, %sample weight loss, and DTG results for untreated brown coal and brown coal treated with Fe and Co additives in accordance with the invention.

### Detailed Description

Thermal analysis methods, such as thermogravimetry (TG), differential thermal analysis (DTA), and differential scanning calorimetry (DSC), have been employed extensively in investigations relating to coal utilization.

Thermogravimetry (TG) is widely used to investigate coal/char reactivity. It is well documented that the reactivity depends on coal rank, maceral composition and/or charring temperature. The coal combustion reactivity was measured by TG, in general, under two conditions (i) isothermal, at a constant temperature, and (ii) non-isothermal, at a constant heating rate. Derivative thermogravimetry (DTG) under non-isothermal conditions, namely burning profile, has been applied to obtain reactivity parameters such as the temperature of maximum (peak) combustion rate (PT), burnt out temperature (BT), and activation energy.

Thermal analysis methods (TGDTA) were used to study the effect of combustion improvers on the kinetic parameters of coal combustion.

### Coal sample specification

The coal used in this study was brown coal from Novomosvsk coal basin.

### Example 1

Iron (II) phthalocyanine (0.1 - 0.2 g) was dissolved in concentrated sulphuric acid (50-60 ml). A sample of brown coal (~ 2 g) (2-3 mm grain size) was stirred in this solution for 2 hours at room temperature and left overnight to soak. After stirring, the coal with the deposited phthalocyanine was filtered off. The residual concentration of iron (II) phthalocyanine was determined by UV/visible spectrophotometric analysis. The quantity of the deposited iron-based additive was determined by the difference in concentrations of the starting and residual solutions. The filtered coal was washed with water to neutral pH and air-dried to constant weight over 72-144 hours. Calculations showed that 0.2% of iron (II) phthalocyanine was deposited on the coal. This corresponds to about 200 ppm of iron. After drying, the sample of coal was ground to dust in a mortar for DTA/DTG analysis.

Comparative measurements were made on untreated ('neat') brown coal and on brown coal treated under the same conditions as for Example 1 but using concentrated sulphuric acid without dissolved iron phthalocyanine ('Fe additive'). Results and calculations are graphed in Figures 1-6 and discussed below.

The DTA results show much higher exothermal activity in the Fe treated sample compared to untreated brown coal. The effect is particularly pronounced around 100 degrees centigrade, between 350 and 450 degrees centigrade, and between 600 and 800 degrees centigrade. Thermal gravimetric measurement was continued to constant weight, with the treated sample losing 91.2% of its initial weight compared to 86.6% for the untreated coal. Furthermore the treated coal reached constant weight at around 800 degrees centigrade, compared to 850 degrees centigrade for the untreated coal. These results demonstrate the additive of the present invention is surprisingly effective in improving the combustion of solid fuels.

### Reaction Model

In treating the obtained DTG data we assumed similarly to the existing literature that the kinetics of coal oxidation is controlled by the first order chemical reaction having the kinetic exponent 0.5<n <1 and that the effect of diffusion can be neglected under the used experimental conditions ${d ⁢ α / d ⁢ τ = k ⁢ \left(1-α\right)}^{n}$
where α is the conversion degree, τ is time, k is the temperature dependent Arrhenius rate constant, k=Aexp(-ΔE^{≠}/RT). R is the gas constant, the model parameters A and ΔE^{≠} are the frequency factor and activation energy. The degree of conversion α is give by the expression α = (mᵢ - m_{τ})/(mᵢ-m_{f}), where mᵢ and m_{f} are the initial and final percent masses and m_{τ} the percent mass at time τ as they are recorded during a TG experiment. The real time and temperature are simply related through the constant heating rate T=T₀+βτ. Assuming n=1 straight lines could be obtained plotting In[-ln(1-α)T²] vs. 1/T. The value of the activation energy could be deduced from the slope of the straight lines obtained.

The first peak around 100 °C corresponds to the loss of the residual water, the second peak at around 300-400 °C corresponds to the release of the volatile matter. In the third stage a sharp peak is observed due to the char combustion,

The obtained activation energy values were as follows.

Brown coal without additives and untreated with H₂SO₄. ΔE^{≠}= 16.8 kJ/mol

Brown coal without additive but treated with H₂SO₄. ΔE^{≠}=16.7 kJ/mol.

Brown coal with Fe additive: DE^{≠}=11.3 kJ/mol.

The use of the Fe additive resulted in a decrease in the energy of activation by
5.5kJ/mol, which is 33% from the initial value of 16.8kJ/mol. Additive testing on brown coal shows improved carbon burnout, resulting in greater total weight loss:

| **Additiive** | **Carbon content ash reduction** |
|---|---|
| Fe Additive | 29% |

The weight loss was achieved at lower temperature, demonstrating the catalytic action of the additive.

| **Additive** | **Total Weight Loss** |
|---|---|
| None | 87.6 % / 850°C |
| Fe Additive | 91.2 % / 800°C |

Linear regression data for Figures 4-6 are set out below in Tables 1-3.

Linear Regression for neat brown coal (Fig. 4): $Y = A + B * X$

**Table 1**

| Parameter | Value | | Error |
|---|---|---|---|
| A | -11.90344 | | 0.06974 |
| B | -2020.06766 | | 59.95073 |
| R | SD | N | P |
| -0.98832 | 0.03655 | 29 | <0.0001 |

Linear Regression for Brown coal with sulphuric acid (Fig. 5): $Y = A + B * X$

**Table 2**

| Parameter | Value | Error |
|---|---|---|
| A | -12.01109 | 0.04844 |
| B | -2008.73036 | 42.37233 |

2

Linear Regression for Brown coal with Fe additive (Fig. 6): $Y = A + B * X$

**Table 3**

| Parameter | Value | | Error |
|---|---|---|---|
| A | -12.69825 | | 0.04571 |
| B | -1359.01275 | | 40,74655 |
| R | SD | N | P |
| -0.98678 | 0.02659 | 32 | <0.0001 |

### Example 2

As for Example 1 but using cobalt phthalocyanine disulphonate as the metal phthalocyanine and distilled water instead of sulphuric acid as the fluid carrier.

Results are shown in Figures 7-11.

While the present invention has been described with reference to specific examples, it should be understood that modifications and variations of the invention may be constructed without departing from the scope of the invention defined in the following claims.

## Claims

1. A method for improving the combustion properties of a coal, the method comprising treating said coal with a metal phthalocyanine.

2. A method according to claim 1, wherein the metal is a transition metal capable of more than one oxidation state.

3. A method according to claim 1 or claim 2, wherein the metal is selected from the group comprising iron, cobalt, manganese or a mixture of all or any two thereof.

4. A method according to any preceding claim, wherein the metal phthalocyanine is iron phthalocyanine.

5. A method according to any preceding claim, wherein the coal is brown coal.

6. A method according to any preceding claim, wherein the step of treating the coal comprises applying to it a solution of the metal phthalocyanine dissolved in a fluid carrier followed by filtering off the solids and drying them or allowing them to dry.

7. A method according to claim 6, further comprising the step of washing the coal with water after removal of the solution.

8. A method according to any of claims 1-5, wherein the step of treating the coal comprises vapour-depositing said metal phthalocyanine.

9. A coal having 0.05-0.5% by wieght of a metal phthalocyanine deposited thereon.

10. A coal according to claim 9, wherein the metal is a transition metal capable of more than one oxidation state.

11. A coal according to claim 9 or claim 10, wherein the metal is selected from the group comprising: iron, cobalt, manganese or a mixture of all or any two thereof.

12. A coal according to any of claims 9-11, wherein the metal phthalocyanine is iron phthalocyanine.

13. A coal according to any of claims 9-12 wherein the coal is brown coal.

14. A method of combustion emission abatement comprising addition of a metal phthalocyanine to coal to form a treated coal, and combusting said treated coal in a combustion chamber with reduction of the excess air in the combustion chamber.

## Patentansprüche

1. Ein Verfahren zur Verbesserung der Verbrennungseigenschaften einer Kohle, wobei das Verfahren ein Behandeln der genannten Kohle mit einem Metall-Phthalocyanin umfasst.

2. Ein Verfahren gemäß Anspruch 1, wobei das Metall ein Übergangsmetall ist, das in der Lage ist, mehr als einen Oxidationszustand einzunehmen.

3. Ein Verfahren gemäß Anspruch 1 oder Anspruch 2, wobei das Metall aus einer Gruppe umfassend Eisen, Kobalt, Mangan oder deren Mischung von allen oder zwei davon ausgewählt ist.

4. Ein Verfahren gemäß einem der vorhergehenden Ansprüche, wobei das Metall-Phthalocyanin ein Eisen-Phthalocyanin ist.

5. Ein Verfahren gemäß einem der vorhergehenden Ansprüche, wobei die Kohle Braunkohle ist.

6. Ein Verfahren gemäß einem der vorhergehenden Ansprüche, wobei der Schritt des Behandelns der Kohle das Einbringen der Kohle in eine Lösung von dem in einem flüssigen Trägersystem gelösten Metall-Phthalocyanin, gefolgt von Abfiltrieren der Feststoffe und Trocknen derselbigen oder Ermöglichen derselbigen zu trocknen, umfasst.

7. Ein Verfahren gemäß Anspruch 6, des Weiteren umfassend den Schritt des Waschens der Kohle mit Wasser nach Entfernung der Lösung.

8. Ein Verfahren nach einem der Ansprüche 1 bis 5, wobei der Schritt des Behandelns der Kohle die Dampfphasenabscheidung des genannten Metall-Phthalocyanins umfasst.

9. Eine Kohle mit darauf abgelagerten 0,05 bis 0,5 Gewichts% eines Metall-Phthalocyanins.

10. Eine Kohle gemäß Anspruch 9, wobei das Metall ein Übergangsmetall ist, das in der Lage ist, mehr als einen Oxidationszustand einzunehmen.

11. Eine Kohle gemäß Anspruch 9 oder 10, wobei das Metall aus einer Gruppe umfassend Eisen, Kobalt, Mangan oder einer Mischung von allen oder zweien davon ausgewählt ist.

12. Eine Kohle gemäß einem der Ansprüche 9 bis 11, wobei das Metall-Phthalocyanin ein Eisen-Phthalocyanin ist.

13. Eine Kohle gemäß einem der Ansprüche 9 bis 12, wobei die Kohle Braunkohle ist.

14. Ein Verfahren zur Herabsetzung der Verbrennungsemission umfassend die Zugabe eines Metall-Phthalocyanins zu Kohle zur Bildung einer behandelten Kohle, und Verbrennen der besagten behandelten Kohle in einer Verbrennungskammer unter Reduzierung von überschüssiger Luft in der Verbrennungskammer.

## Revendications

1. Procédé pour améliorer les propriétés de combustion d'un charbon, le procédé comprenant le traitement dudit charbon avec une phtalocyanine de métal.

2. Procédé selon la revendication 1 où le métal est un métal de transition capable de plus d'un état d'oxydation.

3. Procédé selon la revendication 1 ou la revendication 2 où le métal est choisi dans le groupe comprenant le fer, le cobalt, le manganèse ou un mélange de tous ou deux quelconques de ceux-ci.

4. Procédé selon l'une quelconque des revendications précédentes où la phtalocyanine de métal est la phtalocyanine de fer.

5. Procédé selon l'une quelconque des revendications précédentes où le charbon est du lignite.

6. Procédé selon l'une quelconque des revendications précédentes où l'étape de traitement du charbon comprend l'application à celui-ci d'une solution de la phtalocyanine de métal dissoute dans un vecteur fluide suivie par la séparation des solides par filtration et leur séchage ou le fait de leur permettre de sécher.

7. Procédé selon la revendication 6 comprenant en outre l'étape de lavage du charbon avec de l'eau après retrait de la solution.

8. Procédé selon l'une quelconque des revendications 1-5 où l'étape de traitement du charbon comprend le dépôt en phase vapeur de ladite phtalocyanine de métal.

9. Charbon ayant 0,05-0,5 % en poids d'une phtalocyanine de métal déposée sur lui.

10. Charbon selon la revendication 9 où le métal est un métal de transition capable de plus d'un état d'oxydation.

11. Charbon selon la revendication 9 ou la revendication 10 où le métal est choisi dans le groupe comprenant : le fer, le cobalt, le manganèse ou un mélange de tous ou deux quelconques de ceux-ci.

12. Charbon selon l'une quelconque des revendications 9-11 où la phtalocyanine de métal est la phtalocyanine de fer.

13. Charbon selon l'une quelconque des revendications 9-12 où le charbon est du lignite.

14. Procédé de diminution des émissions de combustion comprenant l'addition d'une phtalocyanine de métal à du charbon pour former un charbon traité, et la combustion dudit charbon traité dans une chambre de combustion avec réduction de l' air en excès dans la chambre de combustion.
